

## UNITED STATES PATENT OFFICE

2,279,560

## VISCOUS HYDROCARBON OIL

Melvin A. Dietrich, Claymont, Del., assignor to  
 E. I. du Pont de Nemours & Company, Wil-  
 mington, Del., a corporation of Delaware

No Drawing. Application May 8, 1940,  
 Serial No. 334,066

5 Claims. (Cl. 252—47)

This invention relates to improved viscous hydrocarbon oils and more particularly to improved lubricating oils and to a process for improving lubricating oils.

The main function of a lubricating oil consists in prevention of seizure of parts, which are in relative motion to one another, through maintenance of a film of lubricant between the moving surfaces. The extent to which this film will be maintained will depend, among other things, on the speed of the moving parts, the bearing pressures, and the temperature. Under present day conditions, particularly in the automotive field, higher speeds, temperatures, and pressures are continually being used with the resultant need for lubricants which will have the necessary film strength to maintain separation of the moving parts, reduce wear, and prevent actual seizure. This may be accomplished by adding to the oil a component which will improve its film strength and load-bearing capacity. A number of materials have been suggested for this purpose, such as esters of long-chain acids, chlorinated hydrocarbons and sulfurized fatty oils. These materials may improve film strength to a certain degree but quite often have objectionable effects along other lines, such as impairing the oxidation resistance of the oil or causing corrosion of bearing metals.

Under conditions of high temperature and exposure to oxygen or air, lubricating oils tend to form corrosive products or sludge which may function adversely on the lubricating efficiency through deposition in oil lines, plugging of oil ducts, formation of deposits on bearing surfaces, or through corrosive action on the engine metals. Although a number of compounds have been suggested for addition to lubricating oils, such as naphthols and secondary or tertiary amines, many of these materials are ineffective at high temperatures or lose their effectiveness in the presence of catalytic metals such as iron or copper.

It is an object of the present invention to improve the properties of viscous hydrocarbon oils. Another object is to improve the stability of viscous hydrocarbon oils. A further object is to improve the film strength and stability of lubricating oils. A still further object is to provide new and improved lubricating oils. Other

objects are to provide new compositions of matter and to advance the art. Still other objects will appear hereinafter.

The above and other may be accomplished in accordance with my invention which comprises incorporating, in a viscous hydrocarbon oil, a small proportion of an organic hydroxamic acid compound of the group of organic hydroxamic acids, organic sulfonhydroxamic acids and the carboxylic acid esters and ethers of said acids. By the addition of such hydroxamic acid compounds to viscous hydrocarbon oils, the stability of such oils against deterioration normally caused by oxygen, heat and the catalytic influence of metals is greatly improved. When the viscous hydrocarbon oil is a lubricating oil which is to be employed for the lubrication of metallic bearing surfaces, it will be found that the hydroxamic acid compounds added in accordance with my invention improve the film strength of such oils.

By the term "viscous" oils, I mean those which have a viscosity of at least 35 seconds Saybolt at 100° F., and intend to include Diesel oils, furnace oils, transformer oils and greases, as well as the ordinary lubricating oils. The oils may be solvent extracted or conventionally refined oils obtained from the various base crude oils. The oils may be employed in greases or may be specially compounded oils such as those containing fish oils, lard oil or castor oil. Preferably the oils are petroleum lubricating oils, that is, lubricating oils derived from petroleum. The improved oils of my invention are preferably employed as lubricants particularly in the lubrication of internal combustion engines, of bearings subjected to high speeds and high pressures, of gears of the hypoid, spiral or bevel types, of railroad rolling stock, and of marine engines. The improved oils of my invention may also be employed as protective coatings for steel and other metal surfaces.

By the term "organic hydroxamic acid," I mean a compound having the formula



wherein R is an organic group having a carbon

atom thereof directly bonded to the carbon of the



By the term "organic sulfonhydroxamic acid," I mean a compound having the formula



wherein R is an organic group having a carbon atom thereof directly bonded to the sulfur of the



By the term "carboxylic acid esters" of such acids, I mean compounds in which the OH of the -NHOH group of the hydroxamic acid or sulfonhydroxamic acid has been esterified with a carboxylic acid. By "ethers" of such acids, I mean compounds in which the hydrogen of the OH group in the -NHOH radical of the hydroxamic or sulfonhydroxamic acid has been replaced by a carbon of an organic group.

While any of the organic hydroxamic acid compounds may be employed, it will generally be preferred that the compounds be devoid of acid substituents. By the term "acid substituents," I mean substituted groups which are acidic in reaction, such as sulfonic acid, carboxylic acid and the like, which would tend to make the compounds acidic in nature, but do intend to include within such term phenolic or alcoholic hydroxy groups or hydroxamic or sulfonhydroxamic acid groups. When I specify that the compound is devoid of acid substituents, I mean that such acid substituents are absent in the neutralized as well as in the unneutralized form.

The organic hydroxamic acids will generally be preferred over the other compounds of the broad class. Such organic hydroxamic acids will preferably contain at least 6 carbon atoms. Amongst the hydroxamic acids, their esters and ethers, those which consist of the elements carbon, hydrogen, oxygen and nitrogen, will be particularly preferred. Of the organic hydroxamic acids, the most desirable will be those which, except for 1 to 2 hydroxamic or



groups, consist of carbon and hydrogen and of these the aliphatic hydroxamic acids, and especially those containing at least 10 carbon atoms, will be preferred. For some purposes, particularly for the stabilization of oils, the dihydroxamic acids and their esters will be preferred. For other purposes, and particularly for producing high film strength, the organic sulfonhydroxamic acids, and particularly the aryl sulfonhydroxamic acids of the benzene series containing one or more alkyl groups on the ring, will be particularly desirable.

Amongst the compounds of my invention, which I have found to be very satisfactory for my purpose, the following are particularly effective:

Laurohydroxamic acid



Sebacodihydroxamic acid



5 Diacetyl ester of adipodihydroxamic acid



10 Dibenzyl ether of adipodihydroxamic acid



15 p-Toluenesulfonhydroxamic acid



20 p-Amylbenzenesulfonhydroxamic acid



25 Oleohydroxamic acid



Palmitohydroxamic acid

30  $\begin{array}{c} \text{O} \\ \parallel \\ \text{C}_{16}\text{H}_{33}-\text{C}-\text{NHOH} \end{array}$

Salicylhydroxamic acid



Adipodihydroxamic acid



Dodecyloxyacetohydroxamic acid



p-tert-Amylphenoxyacetohydroxamic acid



N-dibutylaminoacetohydroxamic acid



Dodecane-1-mercaptopsuccinodihydroxamic acid



Cyclohexylmercaptopsuccinodihydroxamic acid



Beta-phenyladipodihydroxamic acid



## Meta-phenylenedioxyacetohydroxamic acid



## 8(9)-para-hydroxyphenylstearohydroxamic acid



## Stearohydroxamic acid



The organic hydroxamic acid compounds of my invention may be incorporated in the oil by various methods such as by simple mixing and heating where their solubility characteristics permit, or by grinding or passage through a colloid mill as desired. Those of my compounds which contain 6 or more carbon atoms are generally sufficiently soluble so that they may be incorporated by simple mixing and heating. Those having a lower number of carbon atoms are less soluble and would generally require grinding or the like, or the use of a blending agent in order to disperse them in the oil satisfactorily. The concentration of the compounds in the oil will be determined largely by the effect desired, but in general will lie between about 0.1% and about 5%. The preferred concentration will generally be between about 0.2% and about 1.0%. Where it is desired to stabilize the oils against the catalytic effects of metals only, the concentrations of the compound employed may run to 0.01% or even lower depending upon the concentration of metal whose catalytic effect is to be inhibited.

The preparation of hydroxamic acids, their esters, and ethers, is described in the literature and follows well-known chemical methods. The preparation of a few representative compounds is given in the following examples, in which the quantities are given as parts by weight.

## EXAMPLE I

## Preparation of laurohydroxamic acid

27 parts of sodium methylate, contained in 155 parts of methanol solution, was poured into a solution of 35 parts by weight of hydroxylamine hydrochloride in 239 parts of methanol. The sodium chloride was removed and 106 parts of methyl laurate added to the filtrate. After these solutions were thoroughly mixed, an additional 155 parts of the sodium methylate solution was introduced and the mixture allowed to stand at room temperature. After standing 20 hours, the solution was acidified with dilute acetic acid to precipitate the hydroxamic acid. Recrystallization from ethyl acetate gave 98 parts of laurohydroxamic acid, melting at 95° C. N (calculated), 6.51%, N (found), 6.70%.

EXAMPLE II  
Preparation of sebacodihydroxamic acid

A reaction mixture, comprising a methanol solution of diethyl sebacate (258 parts), hydroxylamine (72.6 parts), and sodium methylate (108 parts), was allowed to stand at 30° C. for two days. A stream of dry carbon dioxide gas was then passed through this solution until precipitation of sodium carbonate ceased. The solid was removed by filtration, and the methanol solvent evaporated from the filtrate. After drying, the residue comprised 175 parts of sebacodihydroxamic acid, which was a white solid melting with decomposition at 164° C. N (found), 11.88%; N (calculated), 12.07%.

EXAMPLE III  
Preparation of diacetyl ester of adipodihydroxamic acid

Twenty-five parts of adipodihydroxamic acid was suspended in 207 parts of dioxan at room temperature. Acetic anhydride (31.8 parts) was added with vigorous stirring. The mixture was stirred 15 hours and then refluxed for two hours. After cooling, it was filtered and the solid residue recrystallized from absolute ethyl alcohol. A yield of 16 parts of white product was obtained, M. P. 177.5° C.

EXAMPLE IV  
Preparation of dibenzylether of adipodihydroxamic acid

Twenty-five parts of adipodihydroxamic acid and 39.5 parts of benzyl chloride were distilled into 53.5 parts of methyl alcohol in which 7.2 parts by weight of sodium had been dissolved. The mixture was refluxed 65 hours, diluted with water, and filtered. The solid residue, after crystallization from absolute ethyl alcohol, was white, melted at 137° C., and contained 8.13% nitrogen, compared to a calculated value of 7.87%.

EXAMPLE V  
Preparation of p-toluenesulfonhydroxamic acid

To a solution of 130 parts of hydroxylamine hydrochloride in 400 parts of methanol was added an equivalent amount of sodium methylate in methanol solution followed by 110 parts of p-toluenesulfonyl chloride in 560 parts of methanol. After evaporation of the solvent, the residue was extracted with ether. Repeated recrystallization of the ether-soluble portion from water gave a 10% yield of p-toluenesulfonhydroxamic acid melting at 134° C. Analysis: calc'd. for  $C_7H_9O_3NS$ : S, 17.12%; found: S 17.24%. This melting point is somewhat lower than the one recorded in the literature, namely, 148° C.

The effect of these compounds, on the film strengths of lubricating oils, was determined on two machines, the Cornell friction tester and the Almen machine. The Cornell friction tester consists essentially of a steel pin, held in place by a brass shear pin, which rotates between the flat surfaces of two cylindrical steel blocks. These blocks serve as part of a jaw mechanism which is drawn together at a uniform rate by means of a ratchet and screw during operation, thus applying a continuously increasing load between the steel pin and blocks. The point, at which the lubricating film breaks down sufficiently to per-

mit seizure, is indicated either by the development of a "squeal" or by the shearing of the brass pin. In the following table, the jaw load at point of seizure is given in pounds for the various compounds.

TABLE I  
*Cornell film strength tests*  
(Using a naphthenic base S.A.E. 30 oil)

| Compound                                     | Concen-<br>tration | Load at<br>seizure |
|----------------------------------------------|--------------------|--------------------|
| None—control                                 |                    |                    |
| p-Toluenesulfonhydroxamic acid               | 0.5                | 750                |
| p-Amylbenzenesulfonhydroxamic acid           | 0.5                | 875                |
| Oleohydroxamic acid                          | 0.5                | 1,125              |
| Do.                                          | 1.0                | 1,250              |
| Hydroxamic acids from coconut oil acids*     | 1.0                | 900                |
| Laurohydroxamic acid                         | 1.0                | 950                |
| Palmitohydroxamic acid                       | 1.0                | 350                |
| Salicylhydroxamic acid                       | 1.0                | 4,500+             |
| Sebacodihydroxamic acid                      | 0.5                | 1,325              |
| Adipodihydroxamic acid                       | 0.5                | 1,000              |
| Dodecyloxyacetohydroxamic acid               | 0.5                | 1,150              |
| p-tert-Amyloxyacetohydroxamic acid           | 0.5                | 1,125              |
| N-dibutylaminoacetohydroxamic acid           | 0.5                | 960                |
| Dodecane-1-mercaptopsuccinodihydroxamic acid | 0.5                | 1,100              |
| Cyclohexylmercaptopsuccinodihydroxamic acid  | 0.5                | 900                |
| Beta-phenyladipodihydroxamic acid            | 0.5                | 850                |
| Meta-phenylenedioxoacetohydroxamic acid      | 0.5                | 950                |
| 8(9)-para-Hydroxyphenylstearohydroxamic acid | 0.5                | 900                |
| Dibenzyl ether of adipodihydroxamic acid     | 0.5                | 875                |

\*This is the mixture of hydroxamic acids derived from the mixture of coconut oil acids obtained by hydrolysis of coconut oil.

The Almen machine has been described in Oil and Gas Journal, 30, 109 (1931) and is well known in the industry. Data obtained on this machine are given in Table II.

TABLE II  
*Almen film strength tests*  
(Using an S.A.E. 30 oil of Mid-Continent origin)

| Compound                           | Concen-<br>tration    | Load                      |
|------------------------------------|-----------------------|---------------------------|
| None—control                       |                       |                           |
|                                    | Per cent by<br>weight | Pounds per<br>square inch |
| Laurohydroxamic acid               | 0.025                 | 2,000                     |
|                                    | 0.05                  | 3,500                     |
|                                    | 0.1                   | 5,000                     |
|                                    | 1.0                   | 6,500                     |
| Palmitohydroxamic acid             | 0.5                   | 8,500                     |
| Stearohydroxamic acid              | 0.5                   | 8,500                     |
| Oleohydroxamic acid                | 1.0                   | 6,000                     |
| Naphthenohydroxamic acids*         | 0.5                   | 10,000                    |
|                                    | 1.0                   | 11,000                    |
| p-Toluenesulfonhydroxamic acid     | 0.5                   | 5,500                     |
|                                    | 1.0                   | 8,500                     |
| p-Amylbenzenesulfonhydroxamic acid | 1.0                   | 9,500                     |

\*This is the mixture of hydroxamic acids derived from the mixture of naphthenic acids obtained from petroleum.

In addition to improving film strength, the compounds function as stabilizers in the oil to prevent deterioration of color under oxidizing conditions and in the presence of iron. This beneficial behavior was demonstrated in the following manner: 20 grams of a naphthenic base S. A. E.-30 oil was placed in a 50 cc. Pyrex beaker open to the air at 150° C. for six hours. A piece of autobody steel (1/2" x 1/2") was immersed in the oil during the heating period. Color changes were measured on a Duboscq colorimeter, using the unheated original oil as a standard. From these measurements "% Color Inhibition" was calculated. These data are given in Table III.

TABLE III  
*Color stabilizing action of hydroxamic acids*

| Compound                                 | Concen-<br>tration    | Color<br>inhibition |
|------------------------------------------|-----------------------|---------------------|
| None—control                             | Per cent by<br>weight | Per cent            |
| Laurohydroxamic acid                     | 0.2                   | 63                  |
| Oleohydroxamic acid                      | 0.2                   | 80                  |
| Sebacodihydroxamic acid                  | 0.2                   | 37                  |
| Diacetyl ester of adipodihydroxamic acid | 0.2                   | 80                  |
| Dibenzyl ether of adipodihydroxamic acid | 0.2                   | 56                  |

The effect of this class of compounds on the resistance of lubricating oils to the formation of sludge and degradation products caused by oxidation was determined in the following manner: 20 grams of a paraffin base S. A. E.-20 oil was placed in a 50 cc. beaker, a small piece (1/2" x 1/2") of steel added and the outfit heated in air to a predetermined temperature by immersion in an oil bath. Sludge was determined by diluting 10 grams of oil to 100 cc. volume with special naphtha, chilling at 0° C. for three hours, followed by filtering and weighing the precipitated sludge. The data obtained are given in Table IV.

TABLE IV  
*Sludge formation in oils containing hydroxamic acids*

| Compound                | Cone.                 | Temp.<br>of test | Length<br>of test | Sludge     |
|-------------------------|-----------------------|------------------|-------------------|------------|
| None—control            | Per cent by<br>weight | °C.              | Hours             | Mg./10 gm. |
| Laurohydroxamic acid    | 0.5                   | 170              | 70                | 53.4       |
| Sebacodihydroxamic acid | 0.5                   | 190              | 30                | 32.2       |
| None—control            |                       | 190              | 30                | 44.4       |
| None—control            |                       | 190              | 30                | 14.0       |
| Oleohydroxamic acid     | 0.5                   | 190              | 30                | 48.2       |
| None—control            |                       | 190              | 30                | 29.5       |

It will be noted that the above examples and tests are given for illustration purposes only. It will be readily apparent to those skilled in the art that many variations and modifications can be made, particularly in the compounds employed, the processes of making them, the proportions added to the oils and the conditions of use, without departing from the spirit and scope of my invention, which I intend to claim broadly as in the appended claims. For example, other organic hydroxamic acid compounds which I have found to be satisfactory for my purpose are:

Naphthalodihydroxamic acid



Phenylaminoacetohydroxamic



Acetohydroxamic acid



Butyrohydroxamic acid



## Butylmercaptoacetohydroxamic acid



## Lauroyl ester of acetohydroxamic acid



## Isobutyl ether of adipodihydroxamic acid



## Phenoxyethyl ether of propionohydroxamic acid



## Beta-naphthyoxyacetohydroxamic acid



## o-Methoxybenzohydroxamic acid



Other hydroxamic acids or dihydroxamic acids or their esters or ethers, which will be suitable for use in accordance with my invention, may be derived from the following acids:

| Acids (monobasic)            | Acids (dibasic)                       |
|------------------------------|---------------------------------------|
| Acetic                       | Succinic                              |
| Propionic                    | Malic                                 |
| Butyric                      | Oxalic                                |
| Valeric                      | Beta-methyladipic                     |
| Caprylic                     | Alpha-ethyladipic                     |
| Nonrylic                     | Beta-isopropyladipic                  |
| Capric                       | Beta-tert-butyladipic                 |
| Undecrylic                   | Beta-tert-amyladipic                  |
| Tridecrylic                  | Beta-phenyladipic                     |
| Myristic                     | Beta-(p-hydroxyphenyl)adipic          |
| Pentadecrylic                | Beta-(p-mercaptophenyl)adipic         |
| Margaric                     | Beta-(p-nitrophenyl)adipic            |
| Nonadecrylic                 | Beta-(6-methoxyphenyl)adipic          |
| Arachidic                    | Beta-(p-nitrophenyl)adipic            |
| Cerotic                      | 4-ketopimelic                         |
| Butylmercaptoacetic          | 6-keto-undecanedioic-1,11             |
| Isopropylxyoacetic           | Dodecanedioic-1,12                    |
| Phenylaminocetic             | Dicyclohexanone ketal of muic         |
| Dodeylaminocetic             | Pimelic                               |
| 12-aminostearic              | Suberic                               |
| 12-hydroxystearic            | Azelaic                               |
| 12-hydroxybutyric            | Hexahydroterphthalic                  |
| Alpha-hydroxyvaleric         | Naphthalene-1,8-dicarboxylic          |
| Alpha-chlorostearic          | Dihydronaphthalene-1,4-dicarboxylic   |
| 2,4-dinitrophenyloxyacetic   | Phenylmercaptomalonic                 |
| Cyclohexyloxyacetic          | Alpha-pentadecane-8-mercaptopsuccinic |
| Beta-Naphthyoxyacetic        | Alpha-pentadecyloxy-8-succinic        |
| o-Methoxybenzoic             |                                       |
| p-Ethoxybenzoic              |                                       |
| p-(Butylmercapto)benzoic     |                                       |
| p-(Isopropylmercapto)benzoic |                                       |
| c-(Dimethylamino)benzoic     |                                       |
| m-(Dibutylamino)benzoic      |                                       |
| Dichlorostearic              |                                       |
| Naphthalanemonocarboxylic    |                                       |

In any of the hydroxamic acids, suitable esters and ethers may be used in which the ester or ether radical may be as follows:

| 5 | Ester radicals | 10 | Ether radicals           |
|---|----------------|----|--------------------------|
|   | Acetyl         |    | Phenyl                   |
|   | Propionyl      |    | Ethyl                    |
|   | Butyryl        |    | Propyl                   |
|   | Caprylyl       |    | Butyl                    |
|   | Naphthphenyl   |    | Isobutyl                 |
|   | Lauroyl        |    | Cyclohexyl               |
|   | Oleyl          |    | Naphthyl (alpha or beta) |
|   | Benzoyl        |    | Phenylethyl              |
|   | Cinnamyl       |    | Ethoxyethyl              |
|   | Methacrylyl    |    | Phenoxyethyl             |

15 Mixtures of hydroxamic acids may be used, such as those prepared from mixed acids obtained by saponification of vegetable or animal oils, by oxidation of petroleum hydrocarbons, by oxidation of paraffin wax, or by oxidation of alcohols produced during hydrogenation of carbon oxides.

20 The organic hydroxamic compounds of my invention may be employed in conjunction with other agents, added to the oils for various purposes, such as fatty acid esters, organic phosphites, organic phosphates, halogenated aromatic compounds, pour-point depressants, viscosity index improving agents, anti-ring sticking agents and the like.

25 30 Compositions containing the organic hydroxamic acids are claimed specifically in my copending application Serial No. 334,065 filed on even date herewith.

I claim:

35 1. A composition comprising a major proportion of a viscous hydrocarbon oil having incorporated therein a small proportion of an organic hydroxamic acid compound selected from the group consisting of organic sulfonhydroxamic acids, the carboxylic acid esters and ethers of said acids and carboxylic acid esters and ethers of organic hydroxamic acids.

40 45 2. A composition comprising a major proportion of a viscous hydrocarbon oil having incorporated therein a small proportion of an organic sulfonhydroxamic acid devoid of acid substituents.

3. A composition comprising a major proportion of a viscous hydrocarbon oil having incorporated therein a small proportion of an aromatic sulfonhydroxamic acid devoid of acid substituents.

45 50 4. A composition comprising a major proportion of a viscous hydrocarbon oil having incorporated therein a small proportion of an aryl sulfonhydroxamic acid of the benzene series.

5. A composition comprising a major proportion of a viscous hydrocarbon oil having incorporated therein a small proportion of p-toluene-

60 sulfonhydroxamic acid.

MELVIN A. DIETRICH.